

# United States Patent [19]

Greene

[11] 3,997,423  
[45] Dec. 14, 1976

[54] **SHORT RESIDENCE TIME LOW PRESSURE HYDROPYROLYSIS OF CARBONACEOUS MATERIALS**

3,111,395 11/1963 Sweeney ..... 208/8  
3,839,186 10/1974 Berger ..... 208/8  
3,855,070 12/1974 Squires ..... 208/8

[75] Inventor: **Marvin Greene**, Somerset, N.J.

*Primary Examiner*—Delbert E. Gantz

[73] Assignee: **Cities Service Company**, Tulsa, Okla.

*Assistant Examiner*—James W. Hellwege

[22] Filed: **Oct. 20, 1975**

*Attorney, Agent, or Firm*—John W. Carpenter

[21] Appl. No.: **623,692**

[57] **ABSTRACT**

[52] U.S. Cl. ..... 208/8; 208/11 R;  
208/142

Crushed coal is mixed with hot hydrogen, at 500° to 1,500° C. and 0 to 250 psig., in a reactor, and then, after a short reaction time, rapidly quenched. The total heat-up, reaction, and quench time is less than 2 seconds. This short residence time results in a high yield of coal tars.

[51] Int. Cl.<sup>2</sup> ..... **C10G 1/06**

[58] Field of Search ..... 208/8, 11 R, 142

[56] **References Cited**

**UNITED STATES PATENTS**

3,030,297 4/1962 Schroeder ..... 208/8

**9 Claims, No Drawings**

**SHORT RESIDENCE TIME LOW PRESSURE  
HYDROPYROLYSIS OF CARBONACEOUS  
MATERIALS**

**BACKGROUND OF THE INVENTION**

This invention concerns coal liquefaction. More particularly, it concerns a process for treating coal with hydrogen, in the absence of any added catalyst and/or solvent, to obtain a high yield of coal tars. The utility of the invention resides in the production of high yields of desirable long chain aromatic hydrocarbons from coal.

Processes for treating coal with hydrogen have been known for many years. Prior art references include U.S. Pat. No. 2,658,861; 2,832,724; 3,030,297; and 3,152,063. Typically, these processes have mixed crushed coal with various solvents, with or without added catalyst, and have heated the mixture to reaction temperature, for an extended period of time, in the presence or absence of hydrogen. Such processes have generally given a wide range of products, from gases to light hydrocarbons to high-boiling liquids, in addition to the solid residues. For example, U.S. Pat. No. 3,823,084, issued to W. C. Schroeder on July 9, 1974 discloses mixing coal and hydrogen, in the absence of a solvent, passing the mixture through a bed of hydrogenation catalyst, and recovering liquid and gaseous hydrocarbon products from the product stream. The disadvantages of such processes include addition of a catalyst that will survive the severe reaction conditions, removal of the catalyst from the effluent stream, recovery of a broad spectrum of gaseous, low-boiling and high-boiling liquids, the necessity for solvent addition and removal, and additional processing steps to separate, remove and recycle various portions of the reaction stream.

**SUMMARY OF THE INVENTION**

We believe that we have overcome, or greatly reduced, the disadvantages of prior art processes by our process of treating carbonaceous material with hydrogen, in the absence of added catalyst, with the process comprising the serial steps of (a) adding crushed carbonaceous material to a reactor, (b) adding hot hydrogen to the stream of carbonaceous material, (c) reacting the hydrogen and the carbonaceous material for a period from about 2 milliseconds to less than 2 seconds, and at a pressure between atmospheric and 250 psig, and (d) quenching the mixture within the reactor. In a narrower aspect, the invention concerns a method of converting coal into coal tars, comprising the steps of (a) introducing finely divided coal into a pressure vessel in a continuous stream, and at a pressure between atmospheric pressure and 250 psia, (b) continuously adding hot hydrogen to the pressure vessel so as to impinge and heat said coal stream, (c) limiting contact between the hot hydrogen and the coal stream within the vessel to a period of less than 2 seconds, (d) quenching the hot hydrogen-coal stream with cold hydrogen, within the reactor, and (e) separating coal tars from said quenched hydrogen-coal stream. The separated coal tar stream can then be processed further. The heart of the invention resides in the concept of a short total residence time of the carbonaceous material in the reactor, at a low pressure between about atmospheric pressure and 250 psia, with this residence time including heat-up, reaction, and quench times and coal heat-up rates in excess of 500° C/sec. This short

residence time contrasts sharply with other hydrogenation processes involving catalysts, solvents, and high pressure wherein relatively long residence times are involved and the reaction mixture is quenched outside the reactor.

Our process, involving, at low pressure, short heat-up and quench times, results in improved yields of desirable tar products, no problems of catalyst addition or removal, simplified apparatus, and improved process reliability.

**DETAILED DESCRIPTION OF THE INVENTION**

Feed material for the process broadly includes carbonaceous material, exemplified by coal, lignite, peat, oil shale, tar sands, organic waste, Orinoco tar, gilsonite, and crude oil. A preferred embodiment of the invention uses coal as the solid feed material. It is noted that all of these feed materials, except conventional crude oil, are solids at ambient temperatures.

The solid feed material is crushed to a particle size of less than 1 inch. It is preferred that the particle size be less than about 1/2 inch, and the most preferred particle size is in the range of 50 to 200 mesh (U.S. Sieve).

The process can utilize almost any hydrogen stream as long as the hydrogen content of the stream is sufficient to react with the carbonaceous material and does not contain deleterious components. Broadly, the incoming hydrogen stream can vary from about 30% hydrogen to about 100% hydrogen, based on the partial pressure of hydrogen. Since recycle of a portion of the effluent gas stream is contemplated in the process, the reactant hydrogen stream can also contain components such as methane, propane, and ethane, with these components typically not condensing as they are cooled to quench temperatures.

Since the process involves the mixing and reaction of carbonaceous material and feed hydrogen, the hydrogen-to-carbonaceous material weight ratio is an important consideration. Broadly, this weight ratio can vary from about 0.05 to about 4, with the higher value showing an excess of hydrogen and the lower value resulting in the formation of more char, with reduced amounts of desirable product. A more desirable hydrogen-to-carbonaceous material weight ratio is in the range of from about 0.12 to about 2, and the most preferred ratio is from about 0.6 to about 1.2.

Since an important aspect of this invention resides in the rapid heating and cooling of the reactants and reaction mixture, at low pressure (0-250 psig), respectively, the temperature of the incoming reactants is of some importance. Typically, the temperature of the incoming carbonaceous material is desirably ambient. It is recognized that, due to conduction, radiation and convection from the hot reactor, the incoming feed material may be heated somewhat. Any tendency to overheat the material to near-reaction temperatures can be reduced by various designs to cool the feed material or to move it at such a rate that it does not have time to be heated appreciably.

Prior art processes raise the temperature of the reactants comparatively slowly, such as by using preheaters for the reacting mixture or by heating the reactor externally. Our process is based on heating the reactant hydrogen to above the reaction temperature and then rapidly impinging this hot hydrogen onto the incoming carbonaceous feed material, within the reactor.

The temperature of the incoming hot hydrogen will vary somewhat, depending on the desired hydrogen-to-

carbonaceous material weight ratio of the reactant mixture and upon the desired reaction temperature in the reactor. Typically the inlet hydrogen temperature should be approximately 50° C. higher than the reaction temperature, when the hydrogen-to-carbonaceous material ratio is around 1, with this temperature difference resulting in a rapid heat-up time greater than about 500° C. per second.

Cooling coils may be combined with the mechanical arrangements to reduce the tendency to pre-heat the incoming carbonaceous material. Similarly, the pressure of the incoming hydrogen will exceed that of the reactor. The combination of a slight excess of incoming hydrogen pressure and the weight of the incoming carbonaceous material results in a continuous mass flow of reactants through the reactor.

The reaction temperature can vary from about 400° to about 2000° C., with a preferable range being from about 500° to about 1500° C., and a most preferred range of from about 600° to about 1000° C. The reactor pressure can vary from about 0 to about 250 psig, preferably from about 15 to 150 psig. The total residence time of the reactants in the reactor can vary from about 2 milliseconds to about 2 seconds, preferably from about 5 milliseconds to about 1 second, with a most preferred residence time of from 10 milliseconds to about 900 milliseconds.

This total residence time includes the heatup, reaction and quench times. Since there is reaction between the carbonaceous material and feed hydrogen as soon as the feed materials enter the reactor and are mixed, and since this reaction continues until the quenched mixture exits the reactor, it is difficult to separate the various phases of the total residence time. It is implicit in the invention that the rates of heat-up and quench be rapid. Direct or indirect quench can be used. The heat-up rate of the carbonaceous material is preferably between about 500° C/sec. and 100,000° C/sec.

The quench material added directly can be, broadly, any of a wide variety of gases or liquids that can be added quickly to the reactant mixture in order to cool the mixture below the effective reacting temperature, while the mixture is in the reactor. Materials that are non-reactive with the reactant mixture are preferred, but many common materials can be used. These can include a portion of the recycled gas stream from the process (having components such as methane, ethane, propane), inert gases such as helium or argon, and even such materials as water, nitrogen and CO<sub>2</sub>. Although these latter materials can react at the temperatures found in the reactor, it is understood that these materials can be added to the reactant stream, from the recycle gas stream, at such a temperature and in such volume so that the result is a quenching of the reactant stream, rather than additional reaction between the reactant stream and the quenched material. Hydrogen is thus the preferred quench material, with a process recycle stream rich in hydrogen being a natural extension of the preferred embodiment. Depending upon the reaction temperature and the mass flow through the reactor, a sufficient amount of quenching material, at a suitable temperature, is added to the reactant stream so that the resultant mixture, near the exit of the reactor, has a temperature of about 200°-500° C. The temperature and the amount of quenched material added are sufficient to quench material is naturally higher than that of the pressure within the reactor. Desirably, the quench temperature should be below the effective re-

acting temperature of the components, yet should be high enough to insure that the products of reaction are in the coal tar state, to facilitate downstream separation.

The weight ratio of quench material to product stream is dependent upon such factors as the reaction temperature, components of product stream, excess of hydrogen, and other conditions. Quenching is a function of the sensible heat in the reaction mixture and in the quench stream.

After the quenched reaction mixture departs the reactor, any unreacted solid material, such as ash or char, enters the char pot and is recovered therefrom, while the remainder of the effluent stream, typically predominantly containing coal tars, proceeds to downstream processing units.

Typically, the major products from this process are char, and a high yield of coal tars which include between about 10 and 80 carbon atoms and are predominantly 2-8 attached ring polynuclear aromatics. The constituency of coal tar is well known to those skilled in the art and may be found in such references as The Handbook of Chemistry and Physics, 48th Edition, published by the Chemical Rubber Co. (see page C-12).

The hydrogen used in the process can be obtained from any commercial source, such as char gasification, naphtha and/or methane steam reforming, or cracking of ethane to produce ethylene. The steps of producing, storing, heating, cooling and recycling the hydrogen are well known and need not be discussed here. Reactor design, though an important consideration in terms of economics, is not an essential part of this invention. Any reactor design that will allow for the fast heat-up of the feed carbonaceous material, a short reaction time, and a fast quench of the product stream can be used for the invention.

#### EXAMPLE 1

Illinois No 6 (HvbC), VM MF 36.6%, Ash MF 10.8% Fix. C MF 52.6, ground to 50×100 mesh (U.S.Sieve), was fed to a hydrogenation reactor. The coal assayed 71.2%C, 4.8%H, 1.4%N, 2.9%S, 9.5%O, on moisture-ash-free (MAF) basis. The reactor conditions were 5 psia, 1700° F, H<sub>2</sub> Conc. % 98, Heating rate 160,000° F/SEC, Quench Temp. 400° F, H<sub>2</sub>/Coal, (lb/lb.)1.0, Heat-up Time. (sec.) 0.010, Reaction Time, (sec.) 0.900, and Quench Time (Sec.) 0.020.

Processing and analysis of the reactor effluent, neglecting excess H<sub>2</sub>, gave these results per ton of MAF feed coal;

|                        |          |
|------------------------|----------|
| C                      | 80.5     |
| H                      | 7.0      |
| N                      | 1.2      |
| S                      | 2.0      |
| O                      | 9.2      |
| API Gr.                | -4       |
| Pour Pt. ° F           | 115      |
| Viscosity, SSU         | 1330     |
| HHV, Btu/lb.           | 15050    |
| Metals, ppm            | 600      |
| AST Moist, ° F         |          |
| IBP                    | 450      |
| 50%                    | 900      |
| E.P./% Rec.            | 1100/60% |
| Tar Yield, bbl/ton MAF | 3.3      |

## EXAMPLE 2

Colorado A (HvbB), VM MF 36.8%, Ash MF 8.1%, Fix C MF 55.1, ground to 40×200 mesh (U.S.Sieve), was fed to a hydrogenation reactor. The coal assayed 73.5%C, 5.1%H, 1.6%N, 0.7%S, 11.0%O, on moisture-ash free (MAF) basis. The reactor conditions were 25 psia, 1900° F, H<sub>2</sub> Conc. % 90, Heating rate 120,000° F/SEC, Quench Temp. 350° F, H<sub>2</sub>/Coal, (lb/lb.) 0.50, Heat-up Time, (sec.) 0.015, Reaction Time (sec.) 10 5 0.500, and Quench Time (sec.) 0.010.

Processing and analysis of the reactor effluent, neglecting excess H<sub>2</sub>, gave these results per ton of MAF feed coal;

|                        |         |
|------------------------|---------|
| C                      | 83.6    |
| H                      | 8.3     |
| N                      | 1.1     |
| S                      | 0.4     |
| O                      | 6.6     |
| API Gr.                | -4      |
| Pour Pt. ° F           | 108     |
| Viscosity, SSU         | 1090    |
| HHV, Btu/lb.           | 16000   |
| Metals, ppm            | 350     |
| AST Moist, ° F         |         |
| IBP                    | 460     |
| 50%                    | 920     |
| E.P./% Rec.            | 980/58% |
| Tar Yield, bbl/ton MAF | 3.0     |

## EXAMPLE 3

Utah Hiawatha (HvbB), VM MF 42.5%, Ash MF 5.0%, Fix C MF 52.5 ground to 20×235 mesh (U.S.-Sieve), was fed to a hydrogenation reactor. The coal assayed 77.1%C, 6.2%H, 1.4%N, 0.5%S, 9.8%O, on moisture-ash-free (MAF) basis. The reactor conditions were 10 psia, 1500° F, H<sub>2</sub> Conc.% 85, Heating rate 70,000° F/SEC, Quench Temp. 300° F, H<sub>2</sub>/Coal, (lb/lb.) 2.0, Heat-up Time, (sec.) 0.020, Reaction Time, (sec. 0.100, and Quench Time (sec.) 0.100.

Processing and analysis of the reactor effluent, neglecting excess H<sub>2</sub>, gave these results per ton of MAF feed coal;

|                        |         |
|------------------------|---------|
| C                      | 83.7    |
| H                      | 8.6     |
| N                      | 1.0     |
| S                      | 0.2     |
| O                      | 6.5     |
| API Gr.                | -3      |
| Pour Pt. ° F           | 130     |
| Viscosity, SSU         | 390     |
| HHV, Btu/lb.           | 16500   |
| Metals, ppm            | 190     |
| IBP                    |         |
| 50%                    | 658     |
| E.P./% Rec.            | 720/88% |
| Tar Yield, bbl/ton MAF | 3.0     |

## EXAMPLE 4

Wyoming Big Horn (Sub.B), VM MF 33.9%, Ash MF 18.8%, Fix. C MF 47.3, ground to ~200 mesh (U.S. Sieve), was fed to a hydrogenation reactor. The coal assayed 77.1%C, 6.2%H, 1.4%N, 0.5%S, 9.8%O, on moisture-ash-free (MAF) basis. The reactor conditions were 250 psia, 2250° F, H<sub>2</sub> Conc.% 80, Heating rate 65 60 430,000° F/SEC, Quench Temp. 300° F, H<sub>2</sub>/Coal, (lb/lb.) 3.0, Heat-up Time, (sec.) 0.005, Reaction Time, (sec.) 0.050, and Quench Time (sec.) 0.005.

Processing and analysis of the reactor effluent, neglecting excess H<sub>2</sub>, gave these results per ton of MAF feed coal:

|                        |         |
|------------------------|---------|
| C                      | 82.7    |
| H                      | 8.0     |
| N                      | 1.0     |
| S                      | 0.6     |
| O                      | 7.5     |
| API Gr.                | -4      |
| Pour Pt. ° F           | 120     |
| Viscosity, SSU         | 228     |
| HHV, Btu/lb.           | 15100   |
| Metals, ppm            | 100     |
| AST Moist, ° F         |         |
| IBP                    | 425     |
| 50%                    | 820     |
| E.P./% Rec.            | 850/52% |
| Tar Yield, bbl/ton MAF | 2.5     |

I claim:

1. A process of treating carbonaceous material with hydrogen, in the absence of added catalyst, to produce a yield of carbonaceous tars comprising, in serial combination,
  - a. adding liquid or crushed solid carbonaceous material to a reactor,
  - b. adding hot hydrogen to the stream of carbonaceous material,
  - c. reacting the hydrogen and the carbonaceous material at a pressure between atmospheric pressure and 250 psia, and temperature varying from about 400° to about 2000° C., and
  - d. quenching the mixture, with the total residence time for steps (b) and (c) varying from about 2 milliseconds to about 2 seconds.
2. The process of claim 1, wherein the crushed solid material has an average particle size smaller than about  $\frac{1}{2}$  inch.
3. The process of claim 1, wherein the ratio of carbonaceous material to hydrogen, in the carbonaceous material-hydrogen mixture, varies from about 0.05 to about 4.
4. The process of claim 1, wherein the heat-up time of said carbonaceous material is between about 500° C/sec. and 100,000° C/sec.
5. The process of claim 1, wherein the temperature of the quenched mixture does not exceed about 200° C.
6. The process of claim 1, wherein the quenching material is hydrogen and the carbonaceous material is coal.
7. A method of converting coal into coal tars comprising the steps of:
  - a. introducing finely divided coal into a vessel in a continuous stream, said vessel having a pressure between atmospheric pressure and 250 psia;
  - b. continuously adding hot hydrogen to the vessel so as to impinge said coal stream and effect a reaction with said coal stream at a temperature varying from about 400° to about 2000° C.;
  - c. thereafter quenching the hot hydrogen-coal stream with cold hydrogen with the total residence time of steps b) and c) varying from about 2 milliseconds to about 2 seconds, and
  - d. separating said coal tars from said quenched hydrogen-coal stream.
8. The method of claim 7, wherein
  - a. the coal has an average particle size of less than about  $\frac{1}{2}$  inch,
  - b. the hydrogen/coal weight ratio of the reaction mixture varies from about 0.05 to about 4,

- c. the reaction temperature varies from about 500° to about 1500° C.,
- d. the total residence time of hydrogen and coal is not more than about 1 second,
- e. the cold hydrogen quench stream has a temperature below 200° C., and

- f. the separated liquid hydrocarbon stream is further processed.
9. The method of claim 7, wherein the separated coal tars are further processed, said coal tars having compounds which include between about 10 and 80 carbon atoms.

\* \* \* \* \*

10

15

20

25

30

35

40

45

50

55

60

65